

## UNITED STATES PATENT OFFICE

2,480,845

ELECTROLYTIC REMOVAL OF RESIN  
FROM METALMax Frager and Hyman Iserson,  
Philadelphia, Pa.No Drawing. Application March 14, 1947,  
Serial No. 734,844

6 Claims. (Cl. 204—141)

(Granted under the act of March 3, 1883, as  
amended April 30, 1928; 370 O. G. 757)

1

The invention described and claimed herein may be practiced and used by or for the United States Government for governmental purposes, without payment to us of any royalty therefor.

This invention relates to the removal of films or thin coatings of resin from metallic articles to which they have been applied.

More specifically, this invention relates to the removal of substantially pure thermosetting synthetic plastic resin which has been cured after having been used to coat a steel object, such as a cartridge case for artillery ammunition. This removal is effected (even after the resin has set and hardened on the metal for a long time and at elevated temperatures) by treating the cartridge case or other workpiece in an electrolytic bath in which the workpiece forms the positive pole or anode.

Prior to this invention sand-blasting was the most positive method known for removing such films. Sand-blasting is objectionable, however, because of the resulting surface roughness which occurs and because only a few industrial establishments are equipped to sand-blast work on a production basis at a reasonable cost.

The most satisfactory chemical methods to date have required the use of hot caustic solutions sometimes containing cresylic acid. This type of procedure, however, is not effective with all the phenolic varnish films which are encountered in practice. Other chemical methods have been used by which the use of combinations of caustic solutions and acid treatments has had better success in some cases.

One example of our invention which has been found to be operative in practice is the following:

A steel cartridge case three inches in diameter and bearing a cured coating of unmodified phenol-formaldehyde resin to a thickness of from three to six ten thousandths of an inch is immersed in an electrolytic bath comprising a solution of sodium hydroxide (NaOH flake caustic) (15 parts by weight) and tap water (85 parts by weight). The cartridge case is connected as the positive pole or anode to a source of direct current electricity. As an optimum, a direct current is passed at a current density of from 13 to 27 amperes per square foot. The optimum temperature of the bath is from 200 to 220 degrees Fahrenheit. Treatment for fifteen minutes results in complete removal of the film. Thicker films require a longer treatment. Upon removal of the film, the cartridge case is taken out of the bath. The bath fluid adhering to it is then removed by water rinsing and air drying.

2

The philosophy or mode of operation of the process of this invention appears to be as follows. The caustic attacks or weakens the resin film to some extent. The resin film may have exceedingly minute holes through it. The electric current passes through these holes to the underlying metal. This causes an evolution of gas. The gas in turn peels or strips the residue of the resin film from the metal surface leaving a smooth, clean metal surface which, if it has an oxide film, e. g.,  $Fe_3O_4$ , on it (as a result of anodic treatment), is easily cleaned by ordinary chemical cleaning methods, such as pickling. Obviously such a surface is adapted to receive further plating or other treatment. The  $Fe_3O_4$  coating is useful in providing some measure of corrosion resistance especially when handling or some delay is involved before the work is given additional treatment.

20 It will be readily recognized that there exists a more or less wide range of equivalents for each of the elements or steps of the process of this invention.

For example, the workpiece or core (which is 25 to be cleaned and on which the resin film or coating is located) may be of any metallic substance although this invention is particularly suitable to ferrous metals and alloys.

Similarly, the coating to be removed may be a 30 synthetic plastic capable of forming a thin film as, for example, unmodified, heat reactive, phenol formaldehyde varnish, or a baked varnish film such as those composed of cured thermosetting plastics.

35 This invention is also useful to remove vinyl resins and alkyd resins.

The bath preferably should consist of an alkaline electrolyte, especially one in a higher range of alkalinity. An example of a suitable bath is 40 one containing sodium orthosilicate with or without the addition of a detergent. Although ionizable sodium compounds have been preferred by us, it is obvious that other ionizable compounds, e. g., potassium compounds, would be 45 quite satisfactory. In the use of the potassium basic compounds would prove slightly more effective than that of the sodium because of the higher ionic mobility of the former.

The temperature can be as low as that of the 50 ambient atmosphere or as high as is dictated by the economic limits of heat and pressure which would be required.

Although making the workpiece anodic has been found to be more effective than cathodic 55 electrolysis, the latter is, probably because of the

higher volume of gas evolution, of considerable value in removing the resin films. In the case of cathodic treatment, the film is sufficiently loosened so that it can be readily removed by a strong stream or spray of water or steam or by additional mechanical treatment such as wiping or brushing.

The invention claimed herein is:

1. A method for removing from a metal surface cured thermosetting synthetic plastics in a substantially pure form consisting of unmodified heat reactive resins, which method consists of immersing the workpiece in an electrolytic bath consisting of 15 parts by weight of an alkaline metal hydroxide from the group consisting of sodium and potassium hydroxide and 85 parts by weight of water, and passing a direct current of from 13 to 27 amperes per square foot through said bath and through said workpiece at a temperature of from 200 to 220 degrees Fahrenheit.

2. A method for removing from a metal surface cured thermosetting synthetic plastics in a substantially pure form consisting of unmodified heat reactive resins, which method consists of immersing the workpiece in an electrolytic bath consisting of 15 parts by weight of sodium hydroxide and 85 parts by weight of water, and passing a direct current of from 13 to 27 amperes per square foot through said bath and through said workpiece at a temperature of from 200 to 220 degrees Fahrenheit.

3. A method for removing from a metal surface cured thermosetting synthetic plastics in a substantially pure form consisting of unmodified heat reactive resins, which method consists of immersing the workpiece in an electrolytic bath consisting of 15 parts by weight of potassium hydroxide and 85 parts by weight of water, and passing a direct current of from 13 to 27 amperes per square foot through said bath and through said workpiece at a temperature of from 200 to 220 degrees Fahrenheit.

4. A method for removing from a metal surface cured unmodified heat-reactive phenol formaldehyde coatings, which method consists of immersing the workpiece in an electrolytic bath consist-

ing of 15 parts by weight of an alkaline metal hydroxide from the group consisting of sodium and potassium hydroxide and 85 parts by weight of water, and passing a direct current of from 13 to 27 amperes per square foot through said bath and through said workpiece at a temperature of from 200 to 220 degrees Fahrenheit.

5. A method for removing from a metal surface cured unmodified heat-reactive phenol formaldehyde coatings, which method consists of immersing the workpiece in an electrolytic bath consisting of 15 parts by weight of sodium hydroxide and 85 parts by weight of water, and passing a direct current of from 13 to 27 amperes per square foot through said bath and through said workpiece at a temperature of from 200 to 220 degrees Fahrenheit.

10 6. A method for removing from a metal surface cured unmodified heat-reactive phenol formaldehyde coatings, which method consists of immersing the workpiece in an electrolytic bath consisting of 15 parts by weight of potassium hydroxide and 85 parts by weight of water, and passing a direct current of from 13 to 27 amperes per square foot through said bath and through said workpiece at a temperature of from 200 to 220 degrees Fahrenheit.

20 MAX FRAGER,  
HYMAN ISERSON.

#### REFERENCES CITED

The following references are of record in the file of this patent:

#### UNITED STATES PATENTS

| Number    | Name      | Date         |
|-----------|-----------|--------------|
| 827,802   | Hollis    | Aug. 7, 1906 |
| 1,457,688 | Bohnhardt | June 5, 1923 |

#### OTHER REFERENCES

- "The Cleaning of Metal," by Mitchell (Magnus Chemical Co.), 1930, page 56.  
 "Metal Industry," July 7, 1944, page 8.  
 "Modern Plastics Catalogue," Oct. 1938, table following page 172; Dec. 1941, pages 59, 60, 61.